

## UNITED STATES PATENT OFFICE.

ARLIE W. SCHORGER, OF MADISON, WISCONSIN, ASSIGNOR TO C. F. BURGESS LABORATORIES, INC., OF MADISON, WISCONSIN, A CORPORATION OF DELAWARE.

## METHOD OF MAKING STEREOTYPE MATS.

No Drawing.

Application filed April 9, 1927. Serial No. 182,545.

This invention relates to stereotype mats and is an improvement on the method described in Letters Patent No. 1,524,155, granted to me on January 27, 1925.

5 The rapidity with which modern newspapers are printed is due largely to use of the stereotype mat, also known as a "matrix," or "flong." As soon as a form containing the type has been set up, a stereotype mat is 10 superimposed, then covered with blankets or felts and passed through a rolling machine, whereby the mat acquires a reverse impression of the type. The mat, after drying, is placed in a casting machine where it is held 15 in the form of a cylinder. Molten stereotype metal is now poured into the machine whereby a metal cylinder or semi-circle is obtained containing on its surface an exact duplicate of the type in the original flat form.

20 The stereotype plate is then placed in a cylinder press whereby papers can be printed at high speed. Several casts can be made easily and rapidly from the same mat so that a number of presses can be placed in operation 25 almost simultaneously.

There are two types of stereotype mats in commercial use, the so-called "wet mat" and the "dry mat." The "wet mat," which is in most extensive use, consists of two or three 30 sheets of thin blotting paper and two to four sheets of tissue paper held together by a paste made of starch, dextrin, gum arabic, etc. The tissue is used on the face to obtain a sharp, smooth impression. The wet mat, after having 35 been built up, must be stored in a wet condition. This is a serious objection. Furthermore, it must be dried on the type form as otherwise it would warp and shrink greatly. Considerable labor and much skill, judgment 40 and experience is required to produce a satisfactory wet mat. The rush of work in a newspaper press room cannot tolerate unreliability in the quality of the mats supplied to the casting machine. Without suitable 45 mats the printing cylinders cannot be made and without these the printing cannot proceed. In a modern newspaper office an interruption or even delay incident to bad workmanship on the wet mats, or unreliability in the starch with which they are made is 50 a serious matter. They have to be made up shortly prior to the time fixed for their use and without adequate opportunity for testing, excepting by actual use. But by the 55 time defects in material and workmanship

develop, the harm has been done to the printer and to all those ramifications of the newspaper art which are dependent on the timely issuance of the paper from the press.

The "dry mat" on the other hand, can be 60 stored in the dry state in any quantity, but previous to use must be "conditioned" by being placed in a humidor where it takes up from 10 to 30% of moisture. It is then rolled on the form, removed, placed in a cylindrical 65 "scorcher" where most of the moisture is removed in one or two minutes. It is then ready for use in the casting machine. From the standpoint of initial cost, speed, and ease of manipulation it is preferable to use a dry 70 mat instead of a wet mat. In getting out a "rush" edition where every second counts, it is obvious that greater speed can be obtained with a dry mat.

The objection to the dry mat as now being 75 manufactured is that it has a rougher surface than the wet mat and does not give satisfactory impressions with half-tone blocks with a fine screen, and in general, lacks sharpness of definition. The dry mat does not 80 have the plasticity of a wet mat, so that fractures may be produced during molding on the type, into which the molten stereotype metal will run. On removing the casting, the face 85 of the mat will be torn so that the mat can not be used for a second casting. A properly made mat should permit the making of 10 to 20 casts. The fractures and roughness characteristic of the present dry mat is largely 90 due to the character of the fibres employed. If they are long and the surface roughens readily so that loose fibres are produced, the molten metal will flow amid the fibers, the surface of the mat becoming torn when the casting is removed, so that both the casting 95 and the mat may be rendered useless.

It is not possible to obtain a satisfactory mat by the use of large quantities of adhesives, such as are frequently employed, owing to the fact that the mat when dry is not 100 plastic, and if used wet it has all the disadvantages already pointed out.

With my invention, as will be described below, these objections are overcome by the use of relatively fine, short, soft fibers, formed 105 into a sheet to give an article having a high degree of smoothness, strength and impressionability.

The natural cellulosic fibers available for manufacture of paper are so long and smooth 110

that when a sheet formed from them is subjected to a strain, the fibers either slip past one another or are ruptured. In either case a roughness is produced that permits the metal to run into the surface of the mat. This difficulty cannot be overcome by simply shortening the fibers by cutting, since in this case the sheet would have very little strength. In my process these objections are overcome by cutting and splitting the fibers into fine fibrils. By my method, properly prepared rag stock, cotton linters, wood pulp and similar fibers, either alone or mixed, are placed in a paper-maker's beater or other suitable apparatus, and while suspended in water are subjected to a cutting and splitting action by suitably adjusting the beater roll with respect to the bed plate. After sufficient beating, the original fibers will have been shortened in length and split longitudinally into small fibrils. The splitting action is complete in some fibers; in others the ends are separated into brushes and the fibrils formed on the sides of the fiber given an arborescent appearance. The difference between the fibers before and after beating cannot well be shown in a pen and ink drawing, but is readily apparent under a microscope, particularly, if the fibers are stained in the well known manner. The relatively prolonged beating in water separates the fibers from one another by combing out the pulp and without undue cutting or breakage of the whole fibers develops the fibrillated condition so important to the successful practice of the present invention. Other methods for fibrillating the fibers may be employed. When the fibers are combed out as described above and made into a sheet on the paper machine, the individual fibers are so interlocked by reason of the fibrils that stick out along the sides and ends of the individual fibers that the sheet as a whole acts somewhat like a net, permitting the required amount of stretching and plasticity during molding against the type, but with adequate strength to permit the sheet subsequently to be rolled into cylindrical form and with all the toughness and heat resistance needed for a subsequent repeated contact with hot metal.

In Letters Patent 1,524,155, I follow the operation of beating the fibers by an alkali cooking operation to remove hydrated or gelatinized cellulose which may have formed during the beating operation. This gelatinized cellulose per se is objectionable since, when it dries, it hardens to a horn like brittle mass which shrinks enormously and has a pronounced tendency to warp and curl. The hydrated or gelatinized cellulose may be formed from the pure cellulose fibers themselves after prolonged beating but it is much more readily formed from the various other carbohydrates and gelatinizable materials associated with cellulose fibers in nature. Chemical pulps from wood have a high percentage of such

readily gelatinizable materials present in the form of lignin, hemi-cellulose, hydro-cellulose, and oxycellulose. These forms of cellulosic materials hydrolyze or gelatinize much more readily than the pure or alpha-cellulose fibers when subjected to prolonged beating. The gelatinized cellulose is then easily dissolved or otherwise removed by cooking with an alkaline solution and separated from the purified fiber. The fibrillated fiber remaining is used for making the dry stereotype mat. Wood per se is not used directly as the source of raw material for the beating operation but a chemical wood pulp, such as an easy-bleaching sulphite wood pulp is advantageously used. This preliminary chemical pulping of the wood, well known to those skilled in the art, removes a large percentage of the easily gelatinizable impurities and breaks down the bundles of fibers of the wood so that the fibrillation operation may be more readily performed.

My earlier invention contemplated beating the cellulosic fibers so that these fibers were gelatinized to an appreciable extent upon their exterior surfaces, thereby insuring the removal of practically all of the easily gelatinizable impurities, regardless of whether the raw stock was an impure chemical wood pulp or a purer form of cellulose fiber such as cotton linters. As a result of this excessive beating an alkaline cooking treatment was required in all cases after the beating operation to remove the gelatinized cellulose which causes the dried sheet to become hard, brittle, and have a low receptivity to impression. The fibrillated fibers obtained from the alkaline cook have excellent felting properties with no tendency to become hard or brittle on drying.

In my improved method, the subject of the present specification, I have improved the technique of the process from the standpoint of the manufacturer and have also found that the resulting mat is superior to the mat made by my earlier process in those qualities necessary for the stereotyping art. The present process is much more readily controlled and as a result it is much easier to duplicate results than with my earlier process. I have found that if a cellulose fiber is properly purified of easily gelatinizable materials prior to beating or otherwise treating the fiber to produce fibrillation, it is not necessary to follow the fibrillating operation by an alkaline cook. I have found that sufficient fibrillation may be secured with a minimum amount of gelatinization, whatever gelatinization occurring being insufficient to affect the properties of the resulting mat adversely.

If it is desirable to use cellulose fibers from wood because of their low cost, I have found that the impure fibers may be purified to yield a grade of fibre, high in alpha-cellulose, which may be subjected to a beating opera-

tion without forming an undesirable amount of gelatinized cellulose incident with the desired degree of fibrillation. This pure cellulose thus derived from wood is termed chemically alpha-cellulose. Cotton is composed largely of alpha-cellulose and may be substituted for the alpha-cellulose from wood. In the case of chemical wood pulps, I prefer using fibers so purified that they contain at least 90 per cent alpha-cellulose and preferably 92 per cent or more.

In preparing from wood a pulp high in alpha-cellulose excellent results are obtained by using pulp prepared by the calcium-bisulphite process, technically known as the "sulphite" process. Probably this process is especially suitable since it is effective in removing much of the hemi-cellulose as well as the other impurities from the wood during the cooking operation. The neutral sodium sulphite process is another chemical process which should yield a pulp suited to the making of fibers high in alpha-cellulose. If desired the sulphite or equivalent pulp may be subjected to a bleaching operation previous to cooking with alkali as this facilitates purification. After suitable washing, the pulp is subjected to cooking in an alkali solution to remove a large proportion of the remaining impurities, especially those that are gelatinized readily. With an easy-bleaching sulphite wood-pulp, the alkali cooking solution may properly contain 10% of caustic soda based on the weight of the pulp, and the cooking may be continued until the liquor is no longer alkaline to litmus. The heating or cooking may be performed at atmospheric pressure or at a steam pressure of 5 to 20 pounds. The amount of chemical used and the cooking conditions employed will vary with the nature of the pulp. It will be understood, of course, that other alkalis and alkaline earths may also be employed in the cooking liquor. The resulting fibers, after washing with water, are unchanged in form, softer on drying, are high in alpha-cellulose and have a greatly reduced tendency to gelatinize on beating.

The cooked fibers are thoroughly washed and are then subjected to the previously described beating or other fibrillating operation to secure sufficient fibrillation but without gelatinizing the fibers sufficiently to lower the quality of the stereotype dry mat.

The fibrillated fibers are mixed with a suitable filler, such as a paper maker's clay, and made into mats of the desired thickness, usually 0.030 inch. It is preferable to build up a mat in several layers as this procedure gives greater uniformity and strength. Eight to ten layers have been found very satisfactory. This can be done by the use of various types of paper machines known to those skilled in the art.

The clay impregnates the entire sheet by

filling in the small interstices between the fibers, and the finished mat is strong, flexible and free from crevices. It may be dried and stored like ordinary paper stock, and the quality of any batch may be tested out long in advance of the time for using the batch in commercial press room work.

To put the sheets or mats in condition for any use it is only necessary to bring up their moisture content in a humidor to that content best suited to the needs of the moment. A moisture content of 10 to 30% before "scorching" will be found suitable for most work.

A stereotype mat made as above described even though classifiable as a dry mat and not a wet mat will give clear, deep and sharp impressions having smooth dense surfaces. It may be used for fine line reproductions with much the same results as a wet mat and without any of the worrying uncertainties incident to wet mat production and use.

I claim:

1. The method of making a stereotype dry mat which consists in fibrillating alpha-cellulose, mixing with a filler, and forming into sheets; substantially as described.

2. The method of making a stereotype dry mat which consists in fibrillating cellulosic fibers containing at least 90 per cent of alpha-cellulose and substantially free of readily gelatinizable substances, mixing with a filler and forming into sheets; substantially as described.

3. The method of making a stereotype dry mat which consists in removing substantially all of the readily gelatinizable materials from wood pulp, fibrillating said residual fibers, mixing with a filler and forming into sheets; substantially as described.

4. The method of making a stereotype dry mat which consists in removing substantially all of the readily gelatinizable materials from wood pulp so that the residual fibers will contain at least 92 per cent of alpha-cellulose, fibrillating said residual fibers, mixing with a filler and forming into sheets; substantially as described.

5. The method of making a stereotype dry mat which consists in removing readily gelatinizable materials from chemical wood pulp by cooking said wood pulp in alkali, washing the dissolved materials from the residual fibers, fibrillating said residual fibers, mixing with a filler, and forming into sheets; substantially as described.

6. The method of making a stereotype dry mat which consists in cooking chemical wood pulp with alkali and removing the readily gelatinizable materials from the wood pulp so that the residual fibers will contain at least 90 per cent of alpha-cellulose, fibrillating said residual fibers, mixing with clay and forming into sheets; substantially as described.

7. The method of making a stereotype dry mat which consists in cooking wood to a pulp

in a suitable chemical to dissolve a large part of the hemi-cellulose, washing said pulp with water, cooking in alkali, washing with water, fibrillating said pulp, mixing with a filler and forming into sheets; substantially as described.

8. The method of making a stereotype dry mat which consists in cooking sulphite wood pulp in alkali, washing with water, fibrillating said pulp, mixing with a filler and forming into sheets; substantially as described.

9. The method of making a stereotype dry mat which consists in cooking sulphite wood

pulp in alkali, washing with water, bleaching said washed pulp, fibrillating said bleached pulp, mixing with clay, forming into sheets composed of a plurality of like layers felted together and allowing said sheet to dry; substantially as described.

10. As a step in the manufacture of stereotype dry mats, the process which consists in cooking cellulosic material in alkali to remove gelatinizable substances and then fibrillating, in part at least, the residual cellulosic fibers.

In testimony whereof I affix my signature.  
ARLIE W. SCHORGER.